# EUROPEAN PATENT APPLICATION

(11) **EP 3 783 138 A1**
(43) Date of publication of application: **24.02.2021**
(21) Application number: 20159776.2
(22) Date of filing: 27.02.2020
(51) Int. Cl.: D02G 3/44

(54) **CORE-SPUN YARN, MANUFACTURING METHOD THEREOF AND CUT-RESISTANT PRODUCT**

(30) Priority: 20.08.2019 CN 201910768189
(71) Applicant: Nantong Jiadeli Safety Products Co., Ltd., Nantong, Jiangsu 226000 (CN)
(72) Inventor: FENG, Hua, Nantong, Jiangsu 226000 (CN)
(74) Representative: Vitina, Maruta

(57) **Abstract**

The present invention relates to a core-spun yarn, a manufacturing method thereof and a cut-resistant product. The core-spun yarn comprises a core yarn and a cover yarn covering the core yarn. The core yarn consists of at least two twisted tungsten steel filaments. The cover yarn is latticed after covering the core yarn. The method for manufacturing the core-spun yarn comprises steps of manufacturing core yarns, manufacturing the core-spun yarn, dipping, and drying. In the core-spun yarn provided by the present invention, the core yarn is made of pure tungsten filaments, tungsten steel filaments or tungsten alloy filaments, so the modulus and strength of the core yarn are improved. Moreover, since tungsten is very high in hardness and also thin and light, the inconvenience in use and heaviness are avoided. The obtained core-spun yarn is greatly improved in terms of its cut resistance and can reach the cut levels A4-A9 in the ANSI/ISEA105:2016 standard. Therefore, the cut level of the cut-resistant product prepared from the core-spun yarn of the present invention is improved.

## Description

### TECHNICAL FIELD

The present invention relates to the technical field of yarns, and in particular to a core-spun yarn, a manufacturing method thereof and a cut-resistant product.

### BACKGROUND OF THE PRESENT INVENTION

In recent years, there have been more and more kinds of protective textiles. The protective textiles have been gradually developed toward high-tech industries. This has become an important mark of the progress of the modern textile technology.

At present, there is no deep and systematic study on cut-resistant glove fabric in China. Particularly the analysis on the cut resistance mechanism is far from perfect. For most of the existing cut-resistant gloves, steel filaments or thickening modules are provided in the gloves to enhance the cut resistance of the gloves. However, the gloves prepared by the two methods are inconvenient to wear, uncomfortable to wear, poor in air permeability and non-washable. Some gloves may cause hand skin allergies. Such gloves are unstable in cut resistance and thus not in accordance with the ANSI/ISEA105:2016 standard (cut levels A1 to A9) issued by the American Society for Testing and Materials (ASTM). Additionally, when an object is gripped by a hand wearing such a glove, the object may fall off due to insufficient gripping force, resulting in injuries such as squeezed by the object and hit by the object.

### SUMMARY OF THE PRESENT INVENTION

An objective of the present invention is to provide a core-spun yarn, a manufacturing method thereof and a cut-resistant product, in order to solve the technical defects in the prior art.

For this purpose, the present invention employs the following technical solutions. A core-spun yarn is provided, including a core yarn and a cover yarn covering the core yarn, wherein the core yarn consists of at least two twisted tungsten steel filaments, and the cover yarn is latticed after covering the core yarn.

Further, the tungsten steel filaments are pure tungsten filaments, tungsten steel filaments or tungsten alloy filaments.

Further, the cover yarn is at least one of graphene yarn, carbon fiber, polyethylene fiber, Kevlar fiber, spandex filament, glass fiber, aramid fiber, polyester fiber, polyamide yarn, nylon fiber, polytetrafluoroethylene fiber and polyphenylene sulfide fiber.

Further, the tungsten steel filaments have a diameter of 0.01 mm to 0.06 mm.

Further, the covering approach is double-helical covering or cross covering.

Further, the core-spun yarn further includes a dipped layer which wraps the core-spun yarn.

Further, the at least two twisted tungsten steel filaments account for 20% to 85% of the total weight of the core-spun yarn by weight percentage.

A method for manufacturing a core-spun yarn is provided, including the following steps:
step S1: manufacturing core yarns: manufacturing core yarns from at least two tungsten steel filaments having a diameter of 0.01 mm to 0.06 mm;
step S2: manufacturing a core-spun yarn: manufacturing the core-spun yarn from one of the core yarns obtained in the step S1 and at least two cover yarns by a core-spun yarn process, a twisted yarn process or a covered yarn process;
step S3: dipping: dipping the core-spun yarn obtained in the step S2 in a dipping solution for 5 min to 10 min, wherein the dipping solution is one of butyronitrile, natural latex, waterborne polyurethane and chloroprene rubber; and
step S4: drying: drying the core-spun yarn treated in the step S3.

Further, in the step S2, during the manufacturing of the core-spun yarn, Z-twist and/or S-twist is used, the number of twists of the first cover yarn is 310 to 330, and the number of twists of the second cover yarn is 200 to 220.

A cut-resistant product is provided, which is woven of the core-spun yarn provided by the present invention, wherein the cut-resistant product is a pair of cut-resistant gloves, a cut-resistant backpack or a cut-resistant armguard.

The present invention has the following beneficial effects.
1. In the core-spun yarn provided by the present invention, the core yarn is made of pure tungsten filaments, tungsten steel filaments or tungsten alloy filaments, so the modulus and strength of the core yarn are improved. Moreover, since tungsten is very high in hardness and also thin and light, the inconvenience in use and heaviness are avoided. The obtained core-spun yarn is greatly improved in terms of its cut resistance and can reach the cut levels A4-A9 in the ANSI/ISEA105:2016 standard (cut levels A1 to A9) issued by the American Society for Testing and Materials (ASTM). Therefore, the cut level of the cut-resistant product prepared from the core-spun yarn of the present invention is improved.
2. In the core-spun yarn provided by the present invention, the cover yarn is made of graphene fiber, so the cut-resistant product prepared from the core-spun yarn provided by the present invention is excellent in sweat absorption, quick dry, air permeability, soft texture and high comfortableness.
3. A dipped layer wraps the core-spun yarn provided by the present invention, and the dipped layer is one of butyronitrile, natural latex, waterborne polyurethane and chloroprene rubber. Accordingly, the wear resistance of the core-spun yarn is improved, and the overall structural strength of the core-spun yarn and the cut resistance of the core-spun yarn are enhanced.
4. In addition to good cut resistance, the core-spun yarn provided by the present invention has high tear resistance, good piercing resistance and excellent dimensional stability, and is comfortable to wear, elastic, free of constriction and good in moisture absorption and sweat release effect.

### BRIEF DESCRIPTION OF THE DRAWINGS

Fig. 1 is a flowchart of a method for manufacturing a core-spun yarn according to the present invention;
Fig. 2 is a schematic structure diagram of double-helical covering according to the present invention;
Fig. 3 is a schematic structure diagram of cross covering according to the present invention;
Fig. 4 is a schematic structure diagram of double-helical covering when three core yarns are used in the present invention; and
Fig. 5 is a schematic structure diagram of cross covering when three core yarns are used in the present invention,
in which:
1: core yarn and 2: cover yarn.

### DETAILED DESCRIPTION OF THE PRESENT INVENTION

In order to make the technical problems to be solved, technical solutions and beneficial effects of the present invention clearer, the present invention will be further described below in detail by embodiments. It should be understood that the specific embodiments to be described herein are merely for explaining the present invention, rather than limiting the present invention.

### Embodiment 1

As shown in Figs. 1-5, Embodiment 1 of the present invention provides a method for manufacturing a core-spun yarn, including the following steps.
Step S1: Manufacturing of core yarns: core yarns 1 are manufactured from at least two tungsten steel filaments 11 having a diameter of 0.01 mm.
Step S2: Manufacturing of a core-spun yarn: the core-spun yarn is manufactured from one of the core yarns obtained in the step S1 and two cover yarns 2, where the cover yarns 2 are two graphene yarns. In the covering process, the first graphene yarn is controlled to have 310 twists in Z-twist, and the second graphene yarn is controlled to have 220 twists in S-twist. In the obtained core-spun yarn, in parts by weight, the core yarn accounts for 80% and the two graphene yarns account for 20%.
Step S3: Dipping: the core-spun yarn obtained in the step S2 is dipped in butyronitrile (dipping solution) for 5 min.
Step S4: Drying: the core-spun yarn treated in the step S3 is dried for 10 min.

### Embodiment 2

As shown in Figs. 1-5, Embodiment 2 of the present invention provides a method for manufacturing a core-spun yarn, including the following steps.
Step S1: Manufacturing of core yarns: core yarns 1 are manufactured from at least two tungsten steel filaments 11 having a diameter of 0.025mm.
Step S2: Manufacturing of a core-spun yarn: the core-spun yarn is manufactured from one of the core yarns obtained in the step S1 and two cover yarns 2, where the cover yarns 2 are a graphene yarn and a Kevlar fiber. In the covering process, the graphene yarn is controlled to have 320 twists in Z-twist, and the Kevlar fiber is controlled to have 210 twists in S-twist. In the obtained core-spun yarn, in parts by weight, the core yarn accounts for 70%, the graphene yarn accounts for 10%, and the Kevlar fiber accounts for 10%.
Step S3: Dipping: the core-spun yarn obtained in the step S2 is dipped in waterborne polyurethane (dipping solution) for 6 min.
Step S4: Drying: the core-spun yarn treated in the step S3 is dried for 10 min.

### Embodiment 3

As shown in Figs. 1-5, Embodiment 3 of the present invention provides a method for manufacturing a core-spun yarn, including the following steps.
Step S1: Manufacturing of core yarns: core yarns 1 are manufactured from at least two tungsten steel filaments 11 having a diameter of 0.03 mm.
Step S2: Manufacturing of a core-spun yarn: the core-spun yarn is manufactured from one of the core yarns obtained in the step S1 and two cover yarns 2, where the cover yarns 2 are a graphene yarn and a carbon fiber. In the covering process, the graphene yarn is controlled to have 330 twists in Z-twist, and the second graphene yarn is controlled to have 220 twists in S-twist. In the obtained core-spun yarn, in parts by weight, the core yarn accounts for 85%, the graphene yarn accounts for 10%, and the carbon fiber accounts for 5%.
Step S3: Dipping: the core-spun yarn obtained in the step S2 is dipped in natural latex (dipping solution) for 5 min.
Step S4: Drying: the core-spun yarn treated in the step S3 is dried for 10 min.

### Embodiment 4

As shown in Figs. 1-5, Embodiment 4 of the present invention provides a method for manufacturing a core-spun yarn, including the following steps.
Step S1: Manufacturing of core yarns: core yarns 1 are manufactured from at least two tungsten steel filaments 11 having a diameter of 0.04 mm.
Step S2: Manufacturing of a core-spun yarn: the core-spun yarn is manufactured from one of the core yarns obtained in the step S1 and two cover yarns 2, where the cover yarns 2 are a graphene yarn and a spandex filament. In the covering process, the graphene yarn is controlled to have 310 twists in Z-twist, and the second graphene yarn is controlled to have 220 twists in S-twist. In the obtained core-spun yarn, in parts by weight, the core yarn accounts for 70%, the graphene yarn accounts for 20%, and the spandex filament accounts for 10%.
Step S3: Dipping: the core-spun yarn obtained in the step S2 is dipped in chloroprene rubber (dipping solution) for 5 min.
Step S4: Drying: the core-spun yarn treated in the step S3 is dried for 10 min.

### Embodiment 5

As shown in Figs. 1-5, Embodiment 5 of the present invention provides a method for manufacturing a core-spun yarn, including the following steps.
Step S1: Manufacturing of core yarns: core yarns 1 are manufactured from at least two tungsten steel filaments 11 having a diameter of 0.045mm.
Step S2: Manufacturing of a core-spun yarn: the core-spun yarn is manufactured from one of the core yarns obtained in the step S1 and two cover yarns 2, where the cover yarns 2 are a graphene yarn and a nylon fiber. In the covering process, the graphene yarn is controlled to have 320 twists in Z-twist, and the second graphene yarn is controlled to have 220 twists in S-twist. In the obtained core-spun yarn, in parts by weight, the core yarn accounts for 60%, the graphene yarn accounts for 20%, and the nylon fiber accounts for 20%.
Step S3: Dipping: the core-spun yarn obtained in the step S2 is dipped in waterborne polyurethane (dipping solution) for 5 min.
Step S4: Drying: the core-spun yarn treated in the step S3 is dried for 10 min.

### Embodiment 6

As shown in Figs. 1-5, Embodiment 6 of the present invention provides a method for manufacturing a core-spun yarn, including the following steps.
Step S1: Manufacturing of core yarns: core yarns 1 are manufactured from at least two tungsten steel filaments 11 having a diameter of 0.05 mm.
Step S2: Manufacturing of a core-spun yarn: the core-spun yarn is manufactured from one of the core yarns obtained in the step S1 and two cover yarns 2, where the cover yarns 2 are a graphene yarn and a polyester fiber. In the covering process, the graphene yarn is controlled to have 310 twists in Z-twist, and the second graphene yarn is controlled to have 200 twists in S-twist. In the obtained core-spun yarn, in parts by weight, the core yarn accounts for 55%, the graphene yarn accounts for 30%, and the polyester fiber accounts for 15%.
Step S3: Dipping: the core-spun yarn obtained in the step S2 is dipped in waterborne polyurethane (dipping solution) for 5 min.
Step S4: Drying: the core-spun yarn treated in the step S3 is dried for 10 min.

### Embodiment 7

As shown in Figs. 1-5, Embodiment 7 of the present invention provides a method for manufacturing a core-spun yarn, including the following steps.
Step S1: Manufacturing of core yarns: core yarns 1 are manufactured from at least two tungsten steel filaments 11 having a diameter of 0.06 mm.
Step S2: Manufacturing of a core-spun yarn: the core-spun yarn is manufactured from one of the core yarns obtained in the step S1 and two cover yarns 2, where the cover yarns 2 are a graphene yarn and a polyethylene fiber. In the covering process, the graphene yarn is controlled to have 310 twists in Z-twist, and the second graphene yarn is controlled to have 200 twists in S-twist. In the obtained core-spun yarn, in parts by weight, the core yarn accounts for 55%, the graphene yarn accounts for 30%, and the polyethylene fiber accounts for 15%.
Step S3: Dipping: the core-spun yarn obtained in the step S2 is dipped in waterborne polyurethane (dipping solution) for 5 min.
Step S4: Drying: the core-spun yarn treated in the step S3 is dried for 10 min.

The forgoing description merely shows preferred embodiments of the present invention and is not intended to limit the present invention. Any modification, equivalent replacement or improvement made based on the contents of the specification and drawings of the present invention shall fall into the protection scope of the present invention.

## Claims

1. A core-spun yarn, comprising a core yarn and a cover yarn covering the core yarn, wherein the core yarn consists of at least two twisted tungsten steel filaments, and the cover yarn is latticed after covering the core yarn.

2. The core-spun yarn according to claim 1, wherein the tungsten steel filaments are pure tungsten filaments, tungsten steel filaments or tungsten alloy filaments.

3. The core-spun yarn according to claim 1, wherein the cover yarn is at least one of graphene yarn, carbon fiber, polyethylene fiber, Kevlar fiber, spandex filament, glass fiber, aramid fiber, polyester fiber, polyamide yarn, nylon fiber, polytetrafluoroethylene fiber and polyphenylene sulfide fiber.

4. The core-spun yarn according to claim 1, wherein the tungsten steel filaments have a diameter of 0.01 mm to 0.06 mm.

5. The core-spun yarn according to claim 1, wherein the covering approach is double-helical covering or cross covering.

6. The core-spun yarn according to claim 1, further comprising a dipped layer which wraps the core-spun yarn.

7. The core-spun yarn according to claim 1, wherein the at least two twisted tungsten steel filaments account for 20% to 85% of the total weight of the core-spun yarn by weight percentage.

8. A method for manufacturing a core-spun yarn, comprising the following steps:
step S1: manufacturing core yarns: manufacturing core yarns from at least two tungsten steel filaments having a diameter of 0.01 mm to 0.06 mm;
step S2: manufacturing a core-spun yarn: manufacturing the core-spun yarn from one of the core yarns obtained in the step S1 and at least two cover yarns by a core-spun yarn process, a twisted yarn process or a covered yarn process;
step S3: dipping: dipping the core-spun yarn obtained in the step S2 in a dipping solution for 5 min to 10 min, wherein the dipping solution is one of butyronitrile, natural latex, waterborne polyurethane and chloroprene rubber; and
step S4: drying: drying the core-spun yarn treated in the step S3.

9. The method for manufacturing a core-spun yarn according to claim 8, wherein, in the step S2, during the manufacturing of the core-spun yarn, Z-twist and/or S-twist is used, the number of twists of the first cover yarn is 310 to 330, and the number of twists of the second cover yarn is 200 to 220.

10. A cut-resistant product which is woven of the core-spun yarn according to any one of claims 1 to 6, wherein the cut-resistant product is a pair of cut-resistant gloves, a cut-resistant backpack or a cut-resistant armguard.
